

1,141,719.

A. J. MASKREY,  
METHOD OF OXIDIZING STEEL OR IRON SHEETS.  
APPLICATION FILED OCT. 14, 1913.

Patented June 1, 1915.

2 SHEETS—SHEET 1.



Witnesses:

*J. C. Turner*  
*Elfriede Schmidt.*

Inventor.

*Arthur J. Maskrey*

By *Harry Greese*  
*Attorney.*

1,141,719.

A. J. MASKREY,  
METHOD OF OXIDIZING STEEL OR IRON SHEETS,  
APPLICATION FILED OCT. 14, 1913.

Patented June 1, 1915.  
2 SHEETS—SHEET 2.



*FIG. 4*



Witnesses.

*J. C. Turner*  
*Elfriede Schmidt.*

Inventor.

*Arthur J. Maskrey*

*By Harry Greene*  
*Attorney*

# UNITED STATES PATENT OFFICE.

ARTHUR J. MASKREY, OF CANTON, OHIO, ASSIGNOR OF ONE-HALF TO JOHN E. CARNAHAN, OF CANTON, OHIO.

## METHOD OF OXIDIZING STEEL OR IRON SHEETS.

1,141,719.

Specification of Letters Patent.

Patented June 1, 1915.

Application filed October 14, 1913. Serial No. 795,095.

*To all whom it may concern:*

Be it known that I, ARTHUR J. MASKREY, a citizen of the United States, residing at Canton, in the county of Stark and State 5 of Ohio, have invented a certain new and useful Method of Oxidizing Steel or Iron Sheets, of which the following is a specification.

The invention relates to the oxidation of 10 the surfaces of annealed steel or iron sheets for the purpose of giving them a uniform bluish color. Ordinary processes of annealing such sheets frequently produce a varying color of oxidation thereon merging 15 from a blackish to a dark blue color adjacent to the edges, into a distinctly lighter blue or silvery color in the middle portions of the sheet, which different colors are sometimes emphasized by the subsequent processes in finishing the sheets.

It is believed that the varying color of oxidation from the edges to the middle portions of the sheets is caused largely, if not entirely, by the presence of gases of combustion 25 from the heating furnace which find their way into an ordinary annealing box through the sand luted joints thereof and either form an oxid or a sulfid, depending upon the fuel used, upon the surfaces of the 30 sheets as far inward from the edges thereof as the gases may permeate. And when it has been sought to oxidize separate sheets by a direct or an indirect heat, it has been found that wherever the sheet has been 35 previously handled, the marks of handling will be developed on the surfaces of the sheets along with the oxidation, but of an entirely different and distinct color. This development is caused no doubt by the perspiration 40 from the human hand, and the same difficulty results to a less extent, even though the sheets are handled with gloves.

The object of the present invention is to 45 carry out the annealing process in such a manner as will permit such an oxidation as will give a uniform blue color to the surfaces of the sheets throughout the whole extent thereof, when they are separated after being annealed; and this object is attained by 50 closing a pack of sheets in a retort impervious to the gases of combustion or other heating means, during the annealing process, and then removing the pack from the retort and separating the sheets and exposing 55 them singly while at a red heat to the atmos-

sphere, whereby the surfaces are oxidized to a uniform color.

The annealing process forming part of the improved method, may be performed in an annealing furnace having a retort therein as 60 illustrated in the accompanying drawings, forming part hereof, in which—

Figure 1 is a longitudinal section of the improved annealing furnace; Fig. 2, a plan section thereof on line 2—2, Fig. 1; Fig. 3, 65 a front elevation of the same; and Fig. 4, a transverse section thereof on line 3—3, Fig. 2.

Similar numerals refer to similar parts throughout the drawings.

The retort 1 may be composed of cast metal or other suitably impervious material and should be closed on all sides excepting only at its mouth which is preferably located at one end and is closed by the doors 70

2. Suitable runways 3 are laid in the bottom of the retort and extend forward through the mouth thereof, upon which the carrying plate 4 may be moved into and out of the furnace on the balls 5, which run 75 in the grooves 6 of the runways and the grooves 7 provided on the under side of the carrying plate. The furnace 8 is built around the retort, excepting only the open 80 end thereof, and may be of any suitable construction to properly heat the retort so that its contents may be brought to an annealing 85 temperature of approximately 1400° to 1600° F.

For carrying out the improved process, 90 the sheets are assembled in a pack upon the carrying plate and then run into the retort, as shown in the several figures; after which the doors are closed, or other suitable means are employed for closing the mouth 95 of the retort to retain the heat and exclude an excess of atmospheric air during the annealing process.

The retort is then heated by the furnace or other suitable means, until the sheets in 100 the pack are heated to a uniform temperature for the purpose of annealing, after which the mouth of the retort is opened and the pack of sheets withdrawn therefrom on the carrying plate, and the sheets of the 105 pack are then separated and exposed to the atmosphere while at a red heat, for oxidizing the surfaces.

By heating the sheets in a pack in a retort 110 impervious to the gases of combustion in

the annealing process, it is evident that the edge portions of the sheets will not be discolored by an oxid or a sulfid, as in previous methods of annealing sheets; so that when 5 the pack of sheets is removed from the retort, the edge portions are free from discoloration, and the surfaces of the sheets when separated may be oxidized so as to give them a uniform color throughout the whole 10 extent. And again, it has been found that when sheets are heated in a pack, as herein described, during a considerable period of time, they do not develop upon their surfaces such marks as may be present from 15 handling in previous operations, so that the sheets when finally oxidized, do not show the same; while a single sheet heated to a red heat during a comparatively short space of time, does develop such marks in such a 20 manner as to practically destroy the uniformity of the color thereof when oxidized.

I claim:

1. The process of oxidizing steel or iron sheets consisting in placing a pack of sheets in a retort impervious to the gases of combustion, then heating the sheets in the retort to an annealing temperature, then removing the pack of sheets from the retort and then separately exposing the sheets while heated to an oxidizing agent. 30

2. The process of oxidizing steel or iron sheets consisting in annealing the sheets in a pack in a retort impervious to the gases of combustion, then removing the pack of sheets from the retort and then separately exposing the sheets while heated to an oxidizing agent. 35

ARTHUR J. MASKREY

Witnesses:

ELFRIEDE SCHMIDT,  
CHAS. M. BALL.